

B. F. CLARK.  
LENS GRINDING MACHINE.  
APPLICATION FILED JUNE 3, 1908.

927,949.

Patented July 13, 1909.

4 SHEETS—SHEET 3.



Inventor.  
B. F. Clark.

By.  
Howard P. Johnson  
Attorney

Witnesses.

A. C. Thomas  
W. E. Chene

# UNITED STATES PATENT OFFICE.

CHARLES B. CLARK, OF BANGOR, MAINE.

## PROCESS OF MANUFACTURING WOOD-PULP.

No. 927,950.

Specification of Letters Patent.

Patented July 13, 1909.

Application filed June 12, 1907. Serial No. 378,507.

*To all whom it may concern:*

Be it known that I, CHARLES B. CLARK, of Bangor, in the county of Penobscot and State of Maine, a citizen of the United States, have invented a new and useful Improvement in the Process of Manufacturing Wood-Pulp, of which the following is a full, clear, and exact description, reference being had to the accompanying drawings, forming a 10 part of this specification, in explaining its nature.

My invention relates to the manufacture of wood pulp especially from coniferous, resinous or "fatty" woods and especially 15 also by what is known as the "sulfite process."

The object or objects of my invention are to produce a better pulp by removing from the digester during the process of cooking 20 certain intercellular constituents of the wood or extractives thereof which if left in the digester would tend to injure or detract from the value or quality of the pulp and the paper made from it. By these intercellular 25 constituents or extractives I mean the gummy or resinous matters with other cementing substances that bind the fiber together and I shall refer to the same as extractive matter.

30 It is the further and even more essential object of my invention to provide for the reclamation or saving from the digester of a relatively large amount of the liquor used therein for digesting and which prior to my 35 invention has been allowed to go to waste. By my process I am enabled also to recover from the wood extractive matter of considerable value, in which connection attention 40 is directed to my co-pending application for Letters Patent, Serial No. 378,506, filed June 12, 1907.

I shall describe the different phases of my invention or inventions in the light of the apparatus which thus far I have found most 45 effective in carrying out the process, the construction and arrangement of which apparatus is shown diagrammatically in the drawings.

Referring to the drawings:—A, A<sup>1</sup> are two 50 digesters of ordinary construction which are adapted to become filled with chips. The digesters are supplied with steam by the inlets a in the usual manner. Extending from the top of each of the digesters are 55 pipes a<sup>1</sup> controlled by valves a<sup>2</sup>. These pipes extend from the digesters to pass first

through a cooler B which may be of any suitable construction. From the cooler the pipes extend to connect with a standpipe C which connects with a storage and reclaiming tank 60 D at a point preferably near the bottom thereof.

E is an apparatus for making sulfurous gas and it may be of any known construction. The apparatus E connects by the 65 pipe e with the tank F of a series of tanks F, F<sup>1</sup>, F<sup>2</sup> and F<sup>3</sup> in which the sulfurous gas is mixed with lime water having preferably a high percentage of magnesia. These tanks are connected with one another by a series 70 of pipes f. The lime water by any convenient source of supply, is placed in the upper tank F<sup>3</sup> from which it flows into and through the remaining tanks of the series by means of the connecting pipes before mentioned. So 75 much of the sulfurous gas as is not taken up by the lime water in the tank F passes therefrom by the pipe f<sup>1</sup> into the tank F<sup>2</sup> by a connecting pipe f<sup>2</sup> where it is absorbed.

An exhaust pump G is connected by the 80 pipe g with the tank F<sup>2</sup>, which pump is adapted to establish and maintain circulation in this part of the system. At this point it is to be noted that the means shown 85 for forming sulfurous gas and mixing it with lime water forms no part of my invention, but is one of a number of means or methods, others of which might be employed, as is well known to those versed in the art.

The storage and reclaiming tank D is supplied with the combine or "sulfite liquor" 90 from the tank F by the pipes d which connect with the foot of the standpipe C, which connects, as before described, with the storage tank D. The storage tank D is provided 95 with any suitable vent d<sup>1</sup>. The tank connects from a point at or near its bottom with the two digesters by means of a connecting pipe d<sup>2</sup> and pipes d<sup>3</sup>, d<sup>4</sup>. In the pipes d<sup>3</sup>, d<sup>4</sup> are valves d<sup>4</sup>, d<sup>5</sup> for controlling the supply 100 of liquor from the storage tank to the digesters. A pump H is also placed in the pipe connection between the storage tank and digesters by which the supply from the storage tank may be pumped into the digesters. 105

On one side of the storage tank there is formed an opening therein by which a portion of the contents of the storage tank may be drawn off. The way which I have found the most convenient for doing this is to control the opening in the side of the storage tank by means of a sliding gate d<sup>5</sup> to which 110



gressed that the extractive matter having been extracted has become so changed in character as to injure the pulp or until it has so worked into the digesting liquor or become soluble therein that it is impossible to get it out for reclaiming the liquor, as will hereinafter be explained. It is also apparent that the free relief for taking off the extractive matter should take place as early as possible in order to save as much of the gas-containing liquor as possible for the earlier the liquor is drawn off the more gas will there be in it. To specify in hours and minutes the precise time for the free relief would be impossible inasmuch as pulp-makers carry on the digesting process for various lengths of time; some carry on a rapid process, others cook more slowly. The period of digestion may also vary depending upon the kind of wood used, and the condition of the wood may make a variation in the length of time for carrying on the process of digestion. Owing, therefore, to the nature of the subject, much of the success to be obtained from practicing applicant's process will depend upon the care and skill of the pulp-maker. It might be observed, also, that the free relief from the digester will cause no undue rise in temperature owing especially to the protracted withdrawal of the liquor. There will also be no detrimental fall in the pressure owing to the fact that steam is entering the digester and, as is usually the case, the discharge pipe is smaller than the inlet pipe.

One reason why the constituents and extractives of the wood are especially given up during the period of the free relief is that during this period, by reason of the extraction of a large amount of liquor from the digester, its contents are subjected to violent agitation by the entering steam which tends to disintegrate the fibers of the wood already reduced to a condition where upon such agitation the cellular incrusting and cementing matter of the wood will be given up freely. In other words, during the process of the "cook" by drawing off a large amount of liquor from the digester I tend to cleanse the cellulose of various woody constituents and extractives which if left in the digester would be injurious to the cellulose or pulp.

The time period during which the free relief of the digester continues may, of course, vary depending upon the cooking and rapidity with which the liquor is withdrawn. I prefer that the withdrawal be such that the free relief may be protracted over such a period of time as will enable the extractive matter to be given up so as to pass out of the digester in the removed liquor. Of course this varies depending upon the length and intensity of the cooking. In practice I prefer the free relief to extend over a period of from twenty to forty-five minutes. After the free relief from the digester the cooking

goes on in the liquor left in the tank until a proper reduction of the pulp has been obtained. During this further period of cooking the digester is only relieved of the gas in it. No appreciable amount of liquor will pass over with the gas because on account of the high temperature the process of condensation of steam does not take place so fast.

Thus far by my process I have removed from the digester a large amount of the constituents and extractives of the wood which if left in the digester would be injurious to the cellulose or pulp and which extractive matter is in itself of considerable value. I have also drawn from the digester a large amount of the gas-containing liquor which is valuable for re-use in the digester when clarified of the extractive matter it contains, as may easily be done in the manner now to be described, and which if left in the liquor would tend to seriously damage the pulp at the time of the next cook if the liquor were re-used without clarifying it.

Referring to the method of clarifying or freeing the liquor drawn from the digester into the reclaiming tank of the extractive matter above referred to together with any dirt or other foreign matter which may be contained in the liquor, it will be understood that all the liquor discharged from the digester during the process of cooking is discharged into the storage or reclaiming tank to mingle with the fresh sulfite liquor directed to flow therein as before described. Moreover, by means of the standpipe the old and fresh liquors are mixed with one another before they enter the reclaiming tank. Now I have found that when the new sulfite liquor mingles with the liquor coming from the digester it facilitates the separation of the extractive matter from the main body of liquor in the tank causing the extractive matter to rise to the top of the liquor in the tank and leaving the sulfite liquor below clarified and in condition for re-use in the digester. The separation is also facilitated by agitation and especially if the added liquor is made dense preferably with lime or other matter not injurious to the digesting liquor but strengthening the same, as some gas-absorbing base. It is also desirable if not necessary to a successful accomplishment of the process that the temperature in the reclaiming tank be not too high. If it be too high the gas in the liquor is given up too freely. The temperature which I have found it most advantageous to maintain is one approximating 90 to 100 degrees F. Such temperature is secured by cooling the liquor discharged from the digester and by the added liquor which is cooler than that coming from the digester. While a higher temperature may be more effective in causing a quicker separation of the extractive matter from the sulfite liquor, it is undesirable for the reason that when the

temperature approximates 100 degrees F. the sulfurous gas in the liquor begins to be given up, so in order to keep the gas in the liquor and still facilitate the separation of the extractive matter contained in it I find it desirable to maintain a temperature in the tank approximating 90 to 100 degrees F.

10 The agitation of the liquor in the tank is caused by the pressure of the relief from the digester and in this connection it is to be observed that I prefer to direct the inflow of liquor into the bottom of the tank and in such place and direction that it will cause the liquor to swirl around the sides of the tank.

15 With reference to securing the proper temperature in the tank, this, of course, may be done by any suitable means. I prefer, however, to do it by means of the cooling tank, the arrangement being such that the liquor having passed through it when mixed with 20 the new sulfite liquor will have a temperature substantially that above referred to.

25 The arrangement for obtaining a proper temperature of the liquor passing through the cooler may be obtained by increasing or decreasing the amount of flow of water around the pipes. Of course in passing more water around the pipes of the cooler the liquor when it arrives at the reclaiming tank 30 will be cooler than if a lesser amount of water were passed around the same.

35 After the separation of the extractive matter which rises to the top of the liquor in the reclaiming tank, it may be drawn off by lowering the gate in the side of the tank when the extractive matter will pass over the top 40 of the gate and flow to a point outside the tank. The level of the sulfite liquor in the tank may be determined, or rather the amount of extractive matter to be drawn off 45 may be determined by the gage in the side of the tank. The sulfite liquor being thus relieved of the extractive matter foreign to it may then be pumped back into the digester and used for purposes of cooking as occasion may require.

50 In practice I have found my process a most effective one, for the paper made from the pulp thus obtained is free from the injurious so called "pitch spots" which heretofore have tended to spoil it and caused a serious injury to the manufacturer by reason of the fact that a considerable amount of paper had to be thrown away. I also find that 55 by reclaiming a large amount of the sulfite liquor I make a very material saving in sulfur; in other words, I am enabled to treat wood by the "sulfite process" with an amount of sulfur which has heretofore been 60 considered impossible and from an economical standpoint this saving of sulfur is a very essential item in the manufacture of wood pulp. The extractive matter yields also a further source of revenue.

65 Having thus fully described my invention,

I claim and desire to secure by Letters Patent of the United States:—

1. That improvement in the process of digestively treating wood by the "sulfite process", so called, in a bath of digesting liquor 70 contained in a digester to form wood pulp which consists in removing from the digester during the period of digestion an appreciable quantity of the bath containing resinous matters and extractives of the wood for the 75 purpose of recovering an appreciable portion of the bath after the passing of the resinous matters and extractives into it upon a resolution of the wood, and afterward continuing the process of digestion in the liquor left 80 in the digester.

2. That improvement in the process of digestively treating wood by the "sulfite process", so called, in a bath of digesting liquor 85 contained in a digester to form wood pulp which consists in removing from the digester an appreciable portion of the digesting bath at that time during the period of digestion when the resinous matters and extractives of the wood are being given up to be contained 90 in the removed portion of the bath, and afterward continuing the process of digestion in the liquor left in the digester.

3. That improvement in the process of digestively treating wood by the "sulfite process", so called, in a bath of digesting liquor 95 contained in a digester to form wood pulp which consists in removing from the digester an appreciable portion of the digesting liquor at that time during the period of digestion when the resinous matters and extractives of the wood are being given up most freely to 100 pass into the digesting liquor and afterward continuing the process of digestion in the liquor left in the digester.

4. That improvement in the process of digestively treating wood by the "sulfite process", so called, in a bath of digesting liquor 105 contained in a digester to form wood pulp which consists in removing from the digester during the period of digestion an appreciable portion of the digesting liquor after the passing of the resinous matters and extractives 110 into it upon the resolution of the wood and while such resinous matters and extractives are separable from said removed liquor, and afterward continuing the process of digestion in the liquor left in the digester.

5. That improvement in the process of digestively treating wood by the "sulfite process" 115 in a hot bath of digesting liquor contained in a digester to form wood pulp which consists in removing from the digester an appreciable portion of the digesting liquor at that time during the period of digestion 120 when the resinous matters and extractives of the wood are freely being given up to pass into the removed portion of the bath and before their character has become changed 125 by their cooking long in the hot bath or have 130

become soluble therein, and afterward continuing the process of digestion in the liquor left in the digester.

6. That improvement in the process of digestively treating wood by the "sulfite process" in a bath of digesting liquor contained in a digester to form wood pulp which consists in digestively treating the wood until the digesting liquor in the main body of the 10 digester begins to become changed in color by the resinous matters and extractives of the wood passing into the liquor, then removing from the digester an appreciable portion of the liquor therein containing resinous 15 matters and extractives, the removal to continue for a protracted interval of time, and afterward continuing the process of digestion in the liquor left in the digester.

7. That improvement in the process of digestively treating wood by the "sulfite process" in a bath of digesting liquor contained in a digester to form wood pulp which consists in relieving the digester to obtain therein proper degrees of heat and pressure for digesting until the digesting liquor begins to receive the extracted resinous matters and extractives of the wood as may be noted by the changing color of the liquor, then removing from the digester at the top thereof an 25 appreciable portion of the liquor therein containing extracted resinous matters and extractives, the removal of the liquor from the digester to continue for a protracted interval 30 of time, and afterward continuing the process 35 of digestion in the liquor left in the digester.

8. That improvement in the process of digestively treating wood by the "sulfite process" in a bath of digesting liquor contained in a digester to form wood pulp which consists in removing from the digester an appreciable portion of the liquor therein when the liquor in the body of the digester begins to turn amber color, the removal of the liquor to continue for a protracted interval of time 40 or until the amber-colored liquor becomes 45 dark in color, and afterward continuing the process of digestion in the liquor left in the digester.

9. That improvement in the process of digestively treating wood by the "sulfite process", so called, in a bath of digesting liquor contained in a digester to form wood pulp which consists in slowly raising the temperature of the digester until the temperature 50 therein approximates 290° F., then removing an appreciable quantity of liquor from the digester, the removal of liquor to continue for a protracted interval of time, and afterward continuing the process of digestion in 55 the liquor left in the digester.

10. That improvement in the process of digestively treating wood by the "sulfite process" in a bath of digesting liquor contained in a digester to form wood pulp which consists 60 in a continuation of the process until the res-

inous matters and extractives of the wood are freely being given up to be contained in the digesting liquor as may be noted by the light amber color of the liquor, then removing from the top of the digester an appreciable 70 quantity of the liquor therein, the removal of liquor to continue until the darkening of the amber-colored liquor, and afterward continuing the process in the liquor left in the digester and venting the digester as occasion 75 may require.

11. That improvement in the process of digestively treating wood by the "sulfite process", so called, in a bath of digesting liquor contained in a digester to form wood pulp 80 which consists in removing from the digester during the period of digestion a portion of the digesting liquor containing resinous matters and extractives of the wood separable from the removed liquor, directing the removed 85 liquor to a suitable receptacle and separating the resinous matters and extractives therefrom.

12. That improvement in the process of digestively treating wood by the "sulfite 90 process", so called, in a bath of digesting liquor contained in a digester to form wood pulp which consists in saving by directing to a suitable receptacle gas-containing liquor discharged from the digester during the period of digestion, which liquor contains also 95 resinous matters and extractives of the wood separable from said liquor, and afterward separating the resinous matters and extractives from this saved liquor. 100

13. That improvement in the process of digestively treating wood by the "sulfite process", so called, in a bath of digesting liquor contained in a digester to form wood pulp which consists in saving by directing to 105 a suitable receptacle gas-containing liquor discharged from the digester at that time during the period of digestion when the resinous matters and extractives of the wood are freely passing into the digesting liquor 110 upon a resolution of the wood, and afterward separating the resinous matters and extractives from this saved liquor.

14. That improvement in the process of digestively treating wood by the "sulfite process", so called, in a bath of digesting liquor contained in a digester to form wood pulp which consists in removing from the digester an appreciable portion of the digesting liquor at that time during the period of digestion when the resinous matters and extractives of the wood are freely being given up to pass into the removed portion of the liquor and before their character has become changed by their cooking long in the liquor or have become soluble therein, directing the removed liquor to a suitable receptacle and separating the resinous matters and extractives therefrom.

15. That improvement in the process of

digestively treating wood by the "sulfite process", so called, in a bath of digesting liquor contained in a digester to form wood pulp which consists in saving by directing to a receptacle gas-containing liquor discharged from the digester during the period of digestion which contains resinous matters and extractives separable from said liquor, separating the resinous matters and extractives from the saved liquor by adding other liquor thereto.

16. That improvement in the process of digestively treating wood by the "sulfite process", so called, in a bath of digesting liquor contained in a digester to form wood pulp which consists in saving by directing to a receptacle gas-containing liquor discharged from the digester during the period of digestion which liquor contains resinous matters and extractives separable from said liquor, separating the resinous matters and extractives from the saved liquor by adding thereto a liquor made dense with a gas-absorbing base.

17. That improvement in the process of digestively treating wood by the "sulfite process", so called, in a bath of digesting liquor contained in a digester to form wood pulp which consists in removing from the digester an appreciable portion of the digesting liquor at that time during the period of digestion when the resinous matters and extractives of the wood are freely being given up to pass into the removed portion of the bath and before their character has become changed by their cooking long in the bath or have become soluble therein, separating the resinous matters and extractives from the removed liquor by adding to it fresh liquor.

18. That improvement in the process of digestively treating wood by the "sulfite process", so called, in a bath of digesting liquor contained in a digester to form wood pulp which consists in removing from the digester during the period of digestion a portion of the digesting liquor containing resinous matters and extractives of the wood separable from the removed liquor, cooling the removed liquor directed to a suitable receptacle and separating the resinous matters and extractives therefrom.

19. That improvement in the process of digestively treating wood by the "sulfite process", so called, in a bath of digesting liquor contained in a digester to form wood pulp which consists in saving by directing to a suitable receptacle gas-containing liquor discharged from the digester during the period of digestion, which liquor contains also resinous matters and extractives of the wood separable from said liquor, cooling the saved liquor and afterward separating the resinous matters and extractives therefrom.

20. That improvement in the process of

digestively treating wood by the "sulfite process", so called, in a bath of digesting liquor contained in a digester to form wood pulp which consists in saving by directing to a suitable receptacle gas-containing liquor discharged from the digester at that time during the period of digestion when the resinous matters and extractives of the wood are freely passing into the digesting liquor upon a resolution of the wood, cooling the saved liquor and afterward separating the resinous matters and extractives therefrom.

21. That improvement in the process of digestively treating wood by the "sulfite process", so called, in a bath of digesting liquor contained in a digester to form wood pulp which consists in removing from the digester an appreciable portion of the digesting liquor at that time during the period of digestion when the resinous matters and extractives of the wood are freely being given up to pass into the removed portion of the liquor and before their character has become changed by their cooking long in the liquor or have become soluble therein, cooling the removed liquor directed to a suitable receptacle and separating the resinous matters and extractives therefrom.

22. That improvement in the process of digestively treating wood by the "sulfite process", so called, in a bath of digesting liquor contained in a digester to form wood pulp which consists in removing from the digester during the period of digestion an appreciable portion of the digesting liquor containing resinous matters and extractives of the wood separable from the removed liquor, cooling the removed liquor directed to a suitable receptacle and separating the resinous matters and extractives from the removed liquor by adding other liquor thereto.

23. That improvement in the process of digestively treating wood by the "sulfite process", so called, in a bath of digesting liquor contained in a digester to form wood pulp which consists in saving by directing to a receptacle gas-containing liquor discharged from the digester during the period of digestion which contains resinous matters and extractives separable from said liquor, cooling the saved liquor and afterward separating the resinous matters and extractives therefrom by adding other liquor thereto.

24. That improvement in the process of digestively treating wood by the "sulfite process", so called, in a bath of digesting liquor contained in a digester to form wood pulp which consists in removing from the digester an appreciable portion of the digesting liquor at that time during the period of digestion when the resinous matters and extractives of the wood are freely being given up to be contained in the removed liquor,

cooling the removed liquor directed to a suitable receptacle and separating the resinous matters and extractives from the removed liquor by adding to it other liquor for facilitating such separation.

25. That improvement in the process of digestively treating wood by the "sulfite process", so called, in a bath of digesting liquor contained in a digester to form wood pulp which consists in removing from the digester an appreciable portion of the digesting liquor at that time during the period of digestion when the resinous matters and extractives of the wood are freely being given up to pass into the removed portion of the bath and before their character has become changed by their cooking long in the bath or have become soluble therein, cooling the removed liquor directed to a suitable receptacle and afterward separating the resinous matters and extractives therefrom by adding to the removed liquor fresh liquor.

26. That improvement in the process of

digestively treating wood by the "sulfite process", so called, in a bath of digesting liquor contained in a digester to form wood pulp which consists in removing from the digester an appreciable portion of the digesting liquor at that time during the period of digestion when the resinous matters and extractives of the wood are freely being given up to pass into the removed portion of the bath and before their character has become changed by their cooking long in the bath or have become soluble therein, cooling the removed liquor directed to a suitable receptacle and afterward separating the resinous matters and extractives therefrom by adding fresh liquor thereto directed to flow into said receptacle and rendering the temperature of the combined liquors in the receptacle approximately 90 to 100 degrees F.

CHARLES B. CLARK.

Witnesses:

JOHN E. R. HAYES,  
M. V. FOLEY.